

## UNITED STATES PATENT OFFICE

2,142,120

CREPE THREAD AND FABRIC CONTAINING  
ARTIFICIAL FILAMENTS

Henry Dreyfus, London, and Robert Wighton Moncrieff, Sidney James Menzer and Thomas Eccles, Spondon, near Derby, England, assignors to Celanese Corporation of America, a corporation of Delaware

No Drawing. Application January 31, 1935, Serial No. 4,302. In Great Britain February 8, 1934

20 Claims. (Cl. 117—2)

This invention relates to the manufacture of crepe threads and fabrics, and has for its particular object the production of crepe fabrics of an improved character from threads containing 5 artificial filaments.

Fabrics exhibiting crepe effects have long been obtained by employing in their construction highly twisted threads of natural silk in the gummed state, the crepe effects appearing more particularly when the fabric so formed is subjected to 10 an aqueous scouring treatment. The fabrics obtained by this process are highly valued on account of their pleasing appearance and handle. The production of crepe fabrics in an analogous 15 manner by the use of threads containing artificial filaments has, however, been accompanied by difficulties in various directions, particularly as regards the strength and appearance of the fabrics.

20 It has now been found that considerable improvement can be effected by employing crepe threads containing artificial filaments which have been stretched, i. e. given a permanent elongation. Such stretched threads may be of a cellulose character, or they may consist of organic derivatives of cellulose, for example cellulose acetate or other organic cellulose esters such as cellulose formate, propionate, butyrate, and oxyethyl cellulose acetate, and cellulose ethers such 25 as ethyl and benzyl cellulose.

For example, cellulose acetate threads may be employed which have been stretched to 120, 130, 150, 200, 300, 500% or more of their original length, for example by subjecting them to the 30 action of softening agents such as acetone, or ethylene methylene ether, dioxane and similar cyclic ethers, ethyl or methyl alcohol, or formaldehyde, diluted, if desired, e. g. with water, to bring them into a condition to undergo stretching of the order mentioned. Thus, cellulose acetate threads may with advantage be stretched by about 30% of their original length in the presence of formaldehyde.

Again, there may be employed cellulose derivative threads which have been produced by wet spinning operations in which a high degree of stretch is applied to the extruded filaments during coagulation.

50 Whatever the method employed to stretch the threads, it should be such as to give them a tenacity of at least 2 grams per denier, and preferably more, e. g. 3, 4, or more grams per denier.

Besides considerable fineness of filament denier, cellulose derivative threads stretched as 55 above described have a strength that is of value

when the threads are subjected to the high degree of twisting necessary for the production of crepe effects. But apart from the possibility of stronger crepe threads and fabrics being produced, it is also found that considerable improvement in crepe effect results from the use of such threads, there being obtained a fine, well-marked crepe effect similar to that ordinarily obtained by the use of natural silk crepe threads.

The threads to be stretched may have normal or bright lustre, or they may be threads having a reduced or subdued lustre. For example, where the crepe threads are desired to have a dull appearance, the threads to be treated may with 15 advantage contain a certain amount of pigment, e. g. 1, 2 or 3% of their weight, in accordance with the dullness required. Thus, cellulose acetate threads containing, e. g. in the proportions above indicated, antimony oxide, stannic oxide, 20 or titanium oxide may be employed according to the invention.

The cellulose derivative threads may with advantage be formed from cellulose derivatives of high viscosity characteristics; for example there 25 may be employed cellulose acetate or other cellulose esters as described in U. S. Patent No. 1,708,787. Thus the cellulose acetate should have a viscosity of at least 30 and preferably exceeding 50, for example of the order of 75, 100, 150, or 30 even 200 or more as measured by comparing the viscosity of a 6% solution of the cellulose acetate in acetone with that of glycerine taken as a standard of 100.

After the stretching treatment the threads may 35 then be subjected to a shrinking treatment with the object of restoring in part at least a loss of extensibility resulting from the stretching operation.

The filaments contained in the threads may 40 be continuous or discontinuous in character.

As above stated the stretched threads employed according to the invention may be of a cellulose character, e. g. viscose and nitrocellulose threads. Particularly useful threads are those 45 consisting of regenerated cellulose produced by effecting saponification of cellulose acetate or other cellulose ester threads which have undergone a stretching treatment as above described. Such saponification may be complete or only 50 partial. In partially saponified materials the saponification may be superficial, i. e. the materials may comprise a superficial layer consisting substantially of cellulose or of esters of cellulose of low acyl content, and a core of substantially

unchanged cellulose ester. Such materials are readily obtainable by processes in which cellulose ester materials are impregnated with a saponifying agent, for example aqueous, aqueous-alcoholic, or alcoholic caustic soda during their continuous passage between two points, and are immediately thereafter subjected to elevated temperatures, for instance by passing them over heated drums or the like, so as to effect rapid 10 drying and saponification.

It is in general preferable, however, to employ materials in which saponification has extended considerably below the surface or even throughout the whole section of the material. The 15 saponification may be of a very low order, for example sufficient to produce a loss in weight of 5% or even less. Specially valuable results are obtainable by employing materials which have been saponified so as to effect a loss of weight of 20 between 5 and 20%, and particularly between 8 and 12%. Products of this type in which the saponification extends considerably below the surface or throughout the whole of the material are specially recommended. On the other hand, 25 saponification may be of a much higher order, involving a loss of weight of 30, 40 or even 50% or more, according to the ester content of the initial material, up to complete saponification.

The saponified materials may acquire an affinity 30 for cotton dyestuffs by the saponification treatment which may, or may not, involve loss of affinity for cellulose ester dyes, for example dyes of the dispersed insoluble type. It has been found of particular advantage in connection with 35 cellulose acetate to carry the saponification to such an extent that the material is insoluble in acetone but yet retains a relatively high acetyl content.

The stretched cellulose ester threads which 40 have been completely or partially saponified may consist of materials of high viscosity characteristics or of materials having normal viscosities.

The degree of twist applied to the threads according to the invention may vary within wide 45 limits; for example twist from 45 to 75 or more turns per inch may be applied, it being understood that in general the finer the thread the higher the degree of twist required. Apart from this the degree of twist desirable in any particular case depends upon a number of other 50 factors, including the precise effects required, the material of the filaments, and the fineness of the filaments in the threads. It is to be pointed out in this connection that the fineness of the 55 individual filaments in the threads resulting from the extension effected in the stretching operation is of considerable advantage in bringing out a good crepe effect on the final fabric, as well as lending itself to the production of fabric having 60 a soft handle.

The twist is conveniently applied by means of an apparatus in which the thread is drawn off over the end of a rotating package to a guide substantially in line with the axis of the package, 65 and thereupon led to a take-up device collecting the yarn at a predetermined speed which determines in accordance with the rate of rotation of the package the degree of twist applied. The rotating bobbin may be provided with a flyer to 70 guide the thread from the package, or with advantage the twisting device may be provided with means on an extension of the spindle projecting beyond the package to prevent twist which has been inserted running back to the yarn on the package, as described in U. S. Patent No. 1,784,581.

During twisting the thread may be subjected to the action of wet steam, as by passing it through a steam box disposed between the guide above the spindle and the take-up package. Thread twisted in this way has a final strength 5 considerably higher than that obtained by twisting untreated thread. The tension maintained during twisting may be such as under the action of the applied steam to stretch the thread still further and overcome in part at least the tendency of the thread to increase in denier during twisting. However, even if the twist is allowed to give a denier increase, higher final tenacities are obtained.

The improved crepe threads according to the 15 invention may be applied in any desired manner in the weaving of crepe fabrics either in the weft or warp or both and with any suitable disposition as regards threads having left- and right-hand twists, as for example left- and right-hand twists alternating singly or in pairs in the weft. The threads may also be used otherwise than in woven fabrics; for example, they may be knitted.

What we claim and desire to secure by Letters 25 Patent is:—

1. Process for the production of crepe threads, which comprises stretching cellulose derivative threads in the presence of an organic softening agent for the substance of the threads, and thereafter twisting the threads to a high degree. 30

2. Process for the production of crepe threads, which comprises stretching cellulose acetate threads in the presence of an organic softening agent for the cellulose acetate, and thereafter twisting the threads to a high degree. 35

3. Process for the production of crepe threads, which comprises stretching cellulose acetate threads in the presence of an organic softening agent for the cellulose acetate to give them a tenacity of at least 2 grammes per denier, and thereafter twisting the threads to a high degree. 40

4. Process for the production of crepe threads, which comprises stretching cellulose acetate threads in the presence of an organic softening agent for the cellulose acetate to give them a 45 tenacity of at least 3 grammes per denier, saponifying the threads so as to effect a loss of weight of between 5 and 20% of the cellulose acetate, and thereafter twisting the threads to a high degree.

5. Process for the production of crepe threads, 50 which comprises stretching cellulose derivative threads in the presence of an organic softening agent for the substance of the threads and thereafter twisting the threads to a high degree while applying steam thereto at the point where the twist is inserted.

6. Process for the production of crepe threads, which comprises stretching cellulose acetate threads in the presence of an organic softening agent for the cellulose acetate and thereafter 55 twisting the threads to a high degree while applying steam thereto at the point where the twist is inserted.

7. Process for the production of crepe threads, which comprises stretching cellulose acetate 65 threads in the presence of an organic softening agent for the cellulose acetate to give them a tenacity of at least 2 grammes per denier, and thereafter twisting the threads to a high degree while applying steam thereto at the point where the twist is inserted. 70

8. Process for the production of crepe threads, which comprises stretching cellulose acetate threads in the presence of an organic softening agent for the cellulose acetate to give them a 75

tenacity of at least 3 grammes per denier, saponifying the threads so as to effect a loss of weight of between 5 and 20% of the cellulose acetate, and thereafter twisting the threads to a high degree while applying steam thereto at the point where the twist is inserted.

9. Process for the production of crepe threads, which comprises stretching cellulose acetate threads in the presence of acetone and thereafter twisting the threads to a high degree.

10. Process for the production of crepe threads, which comprises stretching cellulose acetate threads in the presence of dioxane and thereafter twisting the threads to a high degree.

11. Process for the production of crepe threads, which comprises stretching cellulose acetate threads in the presence of formaldehyde and thereafter twisting the threads to a high degree.

12. Process for the production of crepe threads, which comprises stretching cellulose acetate threads by about 30% of their original length in the presence of formaldehyde and thereafter twisting the threads to a high degree.

13. Process for the production of crepe threads, which comprises stretching cellulose ester threads in the presence of an organic softening agent for the substance of the threads, at least partially saponifying the threads, and thereafter twisting the threads to a high degree.

14. Process for the production of crepe threads, which comprises stretching threads of cellulose esters of high viscosity characteristics in the presence of an organic softening agent for the substance of the threads, at least partially saponifying the threads, and thereafter twisting the threads to a high degree.

15. Process for the production of crepe threads, which comprises stretching threads of cellulose acetate of high viscosity characteristics in the presence of an organic softening agent for cellulose acetate, at least partially saponifying the threads, and thereafter twisting the threads to a high degree.

16. Process for the production of crepe threads, which comprises stretching cellulose derivative

threads uniformly along their length and until a permanent elongation is attained in the presence of an organic softening agent for the substance of the threads and thereafter twisting the threads to a high degree.

17. Process for the production of crepe threads, which comprises stretching cellulose acetate threads uniformly along their length and until a permanent elongation is attained in the presence of an organic softening agent for the cellulose acetate to give them a tenacity of at least 2 grams per denier and thereafter twisting the threads to a high degree.

18. Process for the production of crepe threads, which comprises stretching cellulose acetate threads uniformly along their length and until a permanent elongation is attained in the presence of an organic softening agent for the cellulose acetate, saponifying the threads so as to effect a loss of weight between 5 and 20% of the cellulose acetate and thereafter twisting the threads to a high degree.

19. Process for the production of crepe threads, which comprises stretching cellulose derivative threads uniformly along their length and until a permanent elongation is attained in the presence of an organic softening agent for the substance of the threads and thereafter twisting the threads to a high degree while applying steam thereto at the point where the twist is inserted.

20. Process for the production of crepe threads, which comprises stretching cellulose acetate threads uniformly along their length and until a permanent elongation is attained in the presence of an organic softening agent for the cellulose acetate to give the threads a tenacity of at least 3 grams per denier, saponifying the threads so as to effect a loss of weight of between 5 and 20% of the cellulose acetate and thereafter twisting the threads to a high degree while applying steam thereto at the point where the twist is inserted.

HENRY DREYFUS.

ROBERT WIGHTON MONCRIEFF.

SIDNEY JAMES MENZER.

THOMAS ECCLES.

5

15

20

25

30

35

40

45